

# UNITED STATES PATENT OFFICE.

FRITZ KÖRNACHER, OF AUERBACH, GERMANY.

## PROCESS OF MAKING FIRM, ALMOST ENTIRELY WATERPROOF, NON-SLIPPING LEATHER.

1,036,267.

Specification of Letters Patent. Patented Aug. 20, 1912.

No Drawing.

Application filed February 26, 1912. Serial No. 678,807.

*To all whom it may concern:*

Be it known that I, FRITZ KÖRNACHER, manufacturer, citizen of the Empire of Germany, residing at Auerbach, Germany, have 5 invented certain new and useful Improvements in Processes of Making Firm, Almost Entirely Waterproof, Non-Slipping Leather, of which the following is a specification.

It is well known that leather exhibits 10 greater firmness and toughness the less the fibers of the hide are changed or acted on during tanning. It is also known that the firmness of leather may be considerably increased and it may be made very waterproof by being impregnated with substances 15 such as stearin and paraffin.

Various processes for making firm and waterproof leather, adapted to be employed for special purposes are based on these 20 two circumstances, by merely tanning the hide, prepared for the tanning process, by a process (chromo tanning, alum tanning and the like) which has but little action on the hide fibers, and if necessary again tanning with vegetable substances, and after 25 the leather obtained in this manner has been dried, impregnating it with fatty substances or a mixture of such, entire hydrocarbons and the like, under the application of heat.

30 The leather made by this process has, however, the disadvantages of presenting a very ugly, dark, greasy and smeary appearance, and of being only able to be worked with difficulty, and being slippery in use and consequently 35 inapplicable for many purposes. Experiments to avoid these disadvantages by subsequently removing the grease from the surfaces of the leather, always only yield defective results as, owing to the difficulty 40 of this work, either too little grease is dissolved or the solution is too strong, so that the grease is forced fully to the surface and the appearance and quality of the leather is still further affected by having a dark color 45 and soft spongy feel. Under these circumstances it therefore appears quite impossible to improve leather by a subsequent re-tanning with vegetable tanning substances and therefore it has hitherto not been attempted 50 in practice in this case of impregnated leather.

Now this invention relates to a process by means of which all the disadvantages herein before mentioned are removed and

an impregnated, firm or solid leather of 55 unobjectionable appearance is obtained.

This process mainly consists in treating leather, which has been tanned by any suitable method or even only tanned by vegetable substances, and, after being dried, impregnated with saponifiable and unsaponifiable solid substances such as stearin and paraffin, first for 1-3 hours in a solution of an alkaline bath preferably of caustic soda or the like at a strength of 5-10° B., the 60 saponifiable substances found on the surface are saponified and changed, so that they may be removed by a simple washing. The consequence of this is that the leather entirely loses on the outside its greasy character 65 without losing the artificial fullness and firmness imparted to it by the impregnation, and may then be suitably bleached and re-tanned on the surfaces. The extraordinary 70 waterproofness of the leather prevents any 75 damage from the alkali.

The treatment for 1-3 hours of the hides with a sulfuric acid solution of 5-10° B. in strength which then follows, causes the free 80 alkaline salts still contained in or upon the leather and the metal salts derived from the tanning, to be neutralized and rendered non-deleterious and the leather is also thereby thoroughly brightened.

By the double vegetable tanning, that is 85 to say by the double treatment of the raw hides which have been preliminarily tanned with minerals, in vegetable tan liquors and after the impregnation, the leather cuts 90 cleaner and firmer and obtains a rougher surface on the one hand and thus is substantially better adapted for use in shoe or belt factories and on the other hand it greatly assists in producing the appearance desired 95 for these kinds of leather, and finally by the double vegetable tanning namely the preliminary and subsequent tanning, the slipping of the leather when wet is entirely avoided. The final application of the said 100 solutions of metal salts which then takes place, causes the conversion of any soap residues which still remain, into insoluble metal soap, so that the feel of the leather 105 is drier and its firmness and waterproofness is further increased.

The process is carried out approximately as follows: The hides which have been treated as usual are subjected in a raw or

chemically tanned condition to a weak vegetable final tanning. After bleaching and drying, the leather is impregnated by saturating it under the action of heat with 5 saponifiable and unsaponifiable substances together, for instance stearin and paraffin, until it is fully saturated. The leather thus treated is then exposed to the action of alkaline baths, preferably of caustic soda, of 10 a strength of from 5-10° B. in strength, whereupon it is treated with sulfuric acid of 5-10° B. in strength, then again washed, then retanned and finally treated for a short time in a solution of metallic salts, such for 15 instance as alum, aluminum sulfate and the like.

The dressing is done in the ordinary way by drying, pressing, rolling, finishing, etc.

The leather made in this way is extremely 20 firm or solid, and almost perfectly waterproof but dry and clear and from its outside absolutely cannot be differentiated from un-impregnated leather. It may be dyed, fin-

ished and treated exactly like the latter and sized, ribbed and polished, it does not 25 slip when in use, and finally exhibits all the properties which can be called for from a perfectly heavy leather such as sole leather, driving belt leather and saddlery leather.

I declare that what I claim is:

A process for making firm, almost perfectly non-slipping leather from vegetably tanned, or mineralley tanned and vegetably retanned, bleached and dried hides saturated with saponifiable and unsaponifiable fatty 35 substances, such process consisting in treating the leather in an alkaline bath, then washing it, then treating it with sulfuric acid, washing it again, retanning and finally treating it with a solution of metallic salts. 40

In testimony whereof I affix my signature in presence of two witnesses.

FRITZ KORNACHER.

Witnesses:

JEAN GRUND,  
CARL GRUND.